

## UNITED STATES PATENT OFFICE

VICTOR R. ABRAMS, OF BRUNSWICK, GEORGIA, ASSIGNOR TO ARTHUR H. BALLARD, OF  
BRUNSWICK, GEORGIA

## SULPHUR LUBRICANT

No Drawing.

Application filed November 26, 1932. Serial No. 644,503.

My invention aims to provide an improved lubricant and method of producing the same, whereby a stable admixture of free sulphur in a liquid vehicle is made available for lubricating purposes.

As my lubricant is of especial value in the art of cutting and machining metals, I will briefly describe the conditions existing when metal is being cut, for example on a turning 10 lathe, milling machine or the like, in order that the desirability of my lubricant may be better understood. It is found upon examination that the chip curls back over the face of the tool, at a point somewhat back of the 15 cutting edge, and slides away from the cutting edge. The pressure of the chip against the tool face sets up a combination of forces, including compression, tension and shear, which are chiefly responsible for the separation 20 of the chip metal from the stock being operated upon. The tool point or edge proper follows along behind the point of separation and functions chiefly to give a smoothing or burnishing effect to the metal 25 from which the chip has already been separated.

It will thus be evident that the greatest wear on the tool occurs at the point on the face against which the chip bears and that 30 this is behind the edge. At this point the tool is greatly heated owing to the chip sliding along the tool face under the extremely high pressure which necessarily exists and which is chiefly concentrated upon 35 a comparatively small area, resulting in a high degree of friction, and also owing to the compression or deformation which occurs in the chip. If a sufficiently high temperature is permitted to build up, the metal may 40 be unduly upset and result in a rough and torn finished article or machined piece. And of course the friction of chip against tool face causes a cup-shaped depression in the latter which weakens the tool and causes it 45 to fail. Consequently the problem presented is to reduce the friction between the chip and tool face and to prevent the generation of heat to a harmfully high degree.

There exists a space or low pressure region 50 bounded by the tool face, the lower side of the

chip and the surface of the stock being cut, and this space or region facilitates the introduction of a lubricant between the chip and the high pressure area on the tool face and also between the stock and the tool edge. In 55 order to serve as an effective lubricant, the substance used should be such as to maintain lubrication between the frictional surfaces. The more completely a film is maintained, the more perfect will be the lubrication. 60 Other conditions being the same, the ability of a lubricant to maintain a film is largely dependent upon its viscosity at the temperature existing between the bearing surfaces. 65

Unfortunately for their utility as lubricants at elevated temperatures, commercial oils rapidly decrease in viscosity with increase in temperature, and with any of the common lubricating oils used for cutting purposes, irrespective of their viscosity at normal temperatures, the viscosity reaches a very low point when a temperature of 240° to 250° F. has been reached. A measurement of the temperature at the rubbing surface would show a temperature much higher than 70 this. Hence it is that all oils heretofore used in metal cutting have not shown themselves to be much better as lubricants than water or aqueous emulsions. 75

Experiments and tests have shown that 80 free sulphur will serve as a superior cutting lubricant, owing to the fact that at the temperatures involved the sulphur is present between the frictional surfaces as a highly viscous liquid. Sulphur melts at a temperature of 235° F., forming at this temperature a thin, straw-colored liquid. As its temperature is raised, the liquid turns darker and becomes more viscous until at about 370° F. 85 it is so viscous that it can hardly be poured. As the temperature is still further raised, the viscosity decreases, but even at a temperature just below its boiling point (832° F.) it is still much more viscous than is cutting oil at even 240° F. 90

In addition to this property, which greatly assists in maintaining a proper lubricating film between the frictional surface, other properties are possessed by free sulphur 95 which renders it superior to oil or similarly 100

acting lubricants, for metal cutting and other high temperature purposes.

The molten sulphur present at and near the pressure zone not only conducts away 5 heat but the sulphur as it is melted takes up an amount of heat equal to its latent heat of fusion, thus increasing the cooling action.

Furthermore, at the temperatures involved, the sulphur undoubtedly combines 10 with the metal so as to form a sulphide contaminating film, or films, between the surface being lubricated, thereby decreasing the intersurface molecular adhesion and otherwise reducing the friction between chip and tool.

15 I am aware that there are a number of so-called "sulphurized" oils now being used as cutting fluids. These contain in solution sulphur compounds, such as sulphonated mineral or lard oils, or contain elemental sulphur in true solution, and in some cases may also contain small amounts of sulphur particles of colloidal size. I have discovered that finely divided free sulphur (by which 20 I mean sulphur particles of greater than colloidal size) will itself function as a cutting lubricant which is far superior to any of the cutting lubricants containing sulphur in other forms heretofore used, and that this 25 finely divided free sulphur possesses lubricating qualities different from, and in addition to, the qualities possessed by sulphur in other forms. This great superiority becomes the more marked at exceptionally high 30 cutting speeds and when difficultly machinable metals are cut.

35 From a practical standpoint, the sulphur is advantageously in a liquid vehicle, so that it may be readily introduced into the zone 40 of action. If finely divided sulphur (flowers of sulphur) is stirred with oil, water or other liquid vehicles, it will not stay in suspension but will settle out and hence would have to be stirred until almost the time for application 45 in order to be utilized. This is highly inconvenient and therefore impractical as a general proposition.

50 In accordance with my invention, I am able to prepare stable, mobile, admixtures of finely divided sulphur and liquid vehicles, which may contain as much or more than 40% of free sulphur. The great bulk of 55 these sulphur particles, as my product is normally prepared, are greatly above colloidal size, and in practice may be of sufficient size as to be easily visible to the naked eye. The liquid vehicle serves principally as a carrier for the sulphur so that it may be introduced to the zone of lubrication, and 60 does not itself function, except perhaps to a slight incidental degree, as a lubricant.

65 Ordinarily I employ either a low grade, cheap, fuel oil, or simply water, as a vehicle. In order to maintain the sulphur particles, which in practice will be mainly non-col-

oidal in size, in a stable suspension, I employ various "stabilizers", which have the property of actually sustaining the sulphur particles, or causing them to be sustained, in the liquid vehicle or carrier for long periods of time. Although these stabilizing substances do increase the viscosity of the vehicle somewhat, this is purely incidental. The effect with which I am concerned is not that of merely delaying the settling out of the sulphur particles but that of causing them to be sustained for indefinitely long periods of time so as to obtain stable suspensions of free sulphur. By "stable" I do not mean necessarily absolute stability but stability in the sense that there is little or no separation or settling out of the sulphur particles.

70 When I use an oil vehicle for suspending the sulphur particles, I may employ such "stabilizers" as calcium soap, aluminum stearate, zinc stearate, zinc oleate and other metallic soaps, soaps made from soda or lime and fatty acids, rosin soaps, cup grease (which contains soap) and similar substances. When using a water vehicle, I employ such substances for "stabilizers" as starch, gums, dextrin, glue, casein, and the like. These "stabilizers" which I employ may be broadly characterized as being gel-forming materials. The water vehicle type of lubricant is claimed specifically in my co-pending application, Ser. No. 633,541, filed September 16, 1932, as a division in part of my application Ser. No. 603,445, filed April 5, 1932, as a continuation in part of my application Ser. No. 594,741, filed February 23, 1932.

75 Irrespective of what may be the correct explanation for the stabilizing action, I have found in the course of my work that my sulphur mixtures behave as though comprising a discontinuous gelatinous mass composed of particles of elastic gel in contact with each other and having the interspaces containing a liquid, the sulphur particles being distributed between the gel particles and supported thereby. The mass might be termed a "fluid gel", or a "freely flowing gel", because it acts like a liquid which may be 80 readily poured, although largely composed of gel.

85 Upon standing, such mixtures often exude a serum comprised of the liquid contained between the gel particles, forming a layer distinct from the gelatinous mass, the sulphur remaining distributed throughout the latter and stably suspended therein. Gentle agitation or stirring readily causes the serum layer to redistribute itself throughout the gelatinous mass to reform the original mixture.

90 Having discussed the properties and nature of my stable sulphur suspensions, and the theory so far as it is known to me, so that others skilled in the art may be better able 95

to proceed in amplifying the list of sulphur stabilizers which I have specifically named, and in properly using them, I will now describe in detail several particular embodiments of my invention.

*Example 1*

Add about 12% of common soap, such as sodium oleate, to about 88% of a petroleum oil, such as a cheap fuel or engine oil, heat to 300° to 350° F. and agitate until solution is effected. Dilute with petroleum until the resulting solution contains about 1% of soap. Allow to cool, preferably without agitation, and add 5% by weight of powdered commercial sulphur (flowers of sulphur), as by stirring. It may also be found to be advantageous to introduce the sulphur before the final dilution.

The cooling of the solution results in the formation of a gel, which becomes freely flowing upon mixing the sulphur therein. As a result of the mixing, the sulfur particles are coated with soap and this prevents the sulphur from attacking and corroding the metal surfaces with which the lubricant comes in contact during its storage and during its circulation to and from the point where the cutting tool engages the work.

It will be found that for general cutting conditions, a 5% sulphur mixture will make a sufficient lubricant. For lubrication of a hand operated die, for example, only 1% or less by weight of sulphur may be sufficient as the heating is not so great as in the case of machine cutting. Also a smaller percentage may be adequate when the lubricant is not to be reused.

By increasing the soap content, 40% by weight of sulphur may be held stabilized, a mobile paste resulting. The paste may be shipped in cans or other containers, thus effecting a saving in transportation charges, and mixed with oil by the user, so as to secure the desired sulphur percentage for cutting purposes.

It is also possible to make a sulphur cake which is too thick to be poured, or may even be a hard cake, by increasing the soap and sulphur percentages. This can be agitated with oil when it is desired to prepare a lubricant and a stable mixture will result, provided sufficient soap was used in making the cake to insure the proper percentage in the final mixture.

*Example 2*

Add 5 to 10 pounds of hydrated lime to 90 pounds of thin mineral oil, say 24° Bé., stir until the lime is thoroughly wetted and distributed in the oil, and add 5 to 10 pounds of rosin oil of ordinary grade. The mixture may be warmed if desired, but the saponification reaction will take place in the old, being largely completed in a few minutes

and completed in 24 hours. The sustaining power of the mixture may be adjusted by varying the oil percentage, the sustaining power being lessened by increasing the oil concentration. To this mixture is added 5 to 25% powdered sulphur, followed by thorough agitation.

The sulphur will remain in suspension and the entire mixture can be handled in the same manner as an ordinary cutting oil.

Aluminum stearate, cup grease, hard grease, axle grease, or the like, can also be used to modify the stabilizing power of the mixture, as several different stabilizers may be simultaneously employed.

*Example 3*

1% to 5% of starch is mixed with water and the whole heated, as by blowing in steam, to the boiling point. The resulting mixture can be thickened or thinned as desired, and from 5% to 25% of powdered sulphur added. A germicide, or fungicide, such as carbolic acid, may be added to inhibit coagulation of the starch, although the sulphur present may exert a sufficient germicidal effect.

In a modification of this example, glue, dextrin, casein (with alkali) and similar substances may be used in place of starch or mixed with it.

A fatty mineral oil may be added to prevent the lubricant from rusting the iron or steel which is exposed to it, and from 1% to 15% of ordinary soap may be added to increase the wetting of the surface to be lubricated.

From the above examples it will be seen that I have given the art not only a highly superior cutting lubricant but one which is extremely inexpensive to make.

Practical tests have demonstrated that extremely satisfactory results can be secured with my lubricant when operating at high rates of cut. The wear on the tool is much less, the tool maintains its edges for a longer period, and a smoother cut is produced. Tests have shown that tools which would not function with cutting media heretofore employed in the art can be satisfactorily used. Friction and heat are reduced and the operation may be speeded up.

Two instances are given which typify the superior results obtained with my lubricant:

*Drilling Monel metal*

$\frac{1}{8}$ " holes drilled in  $\frac{3}{16}$ " metal. With no lubrication, drill destroyed after  $1\frac{1}{2}$  holes. With regular petroleum lubrication, drill destroyed after 10 holes drilled. With sulphur lubricant in water vehicle (starch stabilizer), the drill was merely dulled after 50 holes.

*Cutting bolts by machine*

Old machine used and with lard oil (considered one of the finest cutting lubricants)

2 to 3 operations required to produce a good thread on  $\frac{3}{4}$ " bolts. Using my sulphur lubricant, the machine was speeded up to maximum speed and only one operation required 5 to give a good thread. One bolt produced per minute as against one per five minutes with lard oil lubrication.

My lubricant is not restricted to cutting operations for the severance of metal, but 10 may be applied advantageously to metal spinning, swaging, drawing and die-pressing operations.

The entire composition (including finely powdered sulphur) can also be used as a 15 lubricant for bearings and frictional surfaces generally and are especially advantageous when the temperatures and pressures are abnormally high. Thus it is very satisfactory for use on hot boxes and on heavy bearings 20 where high temperatures are likely to develop, such as bearings on railway cars, journals, etc., and for heavily loaded gears, particularly of the worm and wheel and hypoid type.

25 By "a freely flowing lubricant" is meant a lubricant which will flow freely at normal temperatures through circulating pipes that are used in the machine tool art for applying cutting fluids to the cutting point, and which 30 is not viscous enough to support sulphur in stable suspension by virtue of the apparent bulk viscosity—in other words, one which is not a paste or a cake.

35 The invention is obviously not restricted to the embodiments described, but what is claimed is as follows:

1. A lubricant for use under extreme-pressure and/or high-temperature conditions comprising a freely flowing discontinuous 40 gelatinous mass composed of particles of elastic gel in contact with each other and having the interspaces containing a liquid of the class typified by oil and water, and a sufficient amount of free sulphur particles of 45 greater than colloidal size to function as a lubricating ingredient distributed between the gel particles and supported thereby.

2. A cutting lubricant comprising a freely flowing discontinuous gelatinous mass composed of particles of elastic gel in contact with each other and having the interspaces containing a liquid of the class typified by oil and water and a sufficient amount of free sulphur particles of greater than 55 colloidal size to function as a lubricating ingredient distributed between the gel particles and supported thereby.

3. The method of preparing a freely flowing lubricant gel containing stably suspended powdered sulphur of greater than colloidal size for use under extreme-pressure and/or high-temperature conditions, comprising heating and mixing together until 60 solution is effected a liquid vehicle of the

class typified by oil and water and a small amount of a suitable elastic-gel-forming substance substantially insoluble therein at normal temperatures, cooling said mixture and allowing a gel to form, and distributing powdered sulphur of greater than colloidal size throughout the gel by mixing therewith, said mixing rendering the gel freely flowing and said gel-forming substance being in sufficient amount to cause said sulphur to be 70 stably suspended.

4. The method of preparing a freely flowing cutting lubricant gel containing stably suspended powdered sulphur of greater than colloidal size, comprising heating and mixing together until solution is effected a liquid vehicle of the class typified by oil and water and a small amount of a suitable elastic-gel-forming substance substantially insoluble therein at normal temperatures, cooling said mixture and allowing a gel to form, and distributing powdered sulphur of greater than colloidal size throughout the gel by mixing therewith, said mixing rendering the gel freely flowing and said gel-forming substance being in sufficient amount to cause said sulphur to be 75 stably suspended.

5. The method of preparing a freely flowing lubricant containing stably suspended free sulphur particles of greater than colloidal size for use under extreme-pressure and/or high-temperature conditions, comprising heating and mixing together until solution is effected a liquid vehicle of the class typified by oil and water and a small amount of a suitable elastic-gel-forming substance substantially insoluble therein at normal temperatures, cooling said mixture and allowing a gel to form, and distributing powdered sulphur of greater than colloidal size throughout the gel by mixing together, said mixing rendering the gel freely flowing and said gel-forming substance being in sufficient amount to cause said sulphur to be 80 stably suspended.

6. The method of preparing a freely flowing cutting lubricant containing stably suspended free sulphur particles of greater than colloidal size, comprising heating and mixing together until solution is effected a liquid vehicle of the class typified by oil and water and a small amount of a suitable elastic-gel-forming substance substantially insoluble therein at normal temperatures, cooling said mixture without agitation until a gel is formed, and distributing powdered sulphur of greater than colloidal size throughout the gel by mixing together, said mixing rendering the gel freely flowing and said gel-forming substance being in sufficient amount to cause said sulphur to be 85 stably suspended.

7. A lubricant for use under extreme-pressure and/or high-temperature conditions comprising a freely flowing discontinuous gelatinous mass composed of particles of

elastic gel in contact with each other and having the interspaces containing oil, and a sufficient amount of free sulphur particles of greater than colloidal size to function as a lubricating ingredient distributed between the gel particles and supported thereby.

8. A cutting lubricant comprising a freely flowing discontinuous gelatinous mass composed of particles of elastic gel in contact with each other and having the interspaces containing oil and a sufficient amount of free sulphur particles of greater than colloidal size to function as a lubricating ingredient distributed between the gel particles and supported thereby.

9. The method of preparing a freely flowing lubricant gel containing stably suspended powdered sulphur of greater than colloidal size for use under extreme-pressure and/or high-temperature conditions, comprising heating and mixing together until solution is effected an oil vehicle and a small amount of a suitable elastic-gel-forming substance substantially insoluble therein at normal temperatures, cooling said mixture and allowing a gel to form, and distributing powdered sulphur of greater than colloidal size throughout the gel by mixing therewith, said mixing rendering the gel freely flowing and said gel-forming substance being in sufficient amount to cause said sulphur to be stably suspended.

10. The method of preparing a freely flowing cutting lubricant gel containing stably suspended powdered sulphur of greater than colloidal size, comprising heating and mixing together until solution is effected an oil vehicle and a small amount of a suitable elastic-gel-forming substance substantially insoluble therein at normal temperatures, cooling said mixture and allowing a gel to form, and distributing powdered sulphur of greater than colloidal size throughout the gel by mixing therewith, said mixing rendering the gel freely flowing and said gel-forming substance being in sufficient amount to cause said sulphur to be stably suspended.

11. The method of preparing a freely flowing lubricant containing stably suspended free sulphur particles of greater than colloidal size for use under extreme-pressure and/or high-temperature conditions, comprising heating and mixing together until solution is effected an oil vehicle and a small amount of a suitable elastic-gel-forming substance substantially insoluble therein at normal temperatures, cooling said mixture without agitation until a gel is formed, and distributing powdered sulphur of greater than colloidal size throughout the gel by mixing together, said mixing rendering the gel freely flowing and said gel-forming substance being in sufficient amount to cause said sulphur to be stably suspended.

12. The method of preparing a freely flow-

ing cutting lubricant containing stably suspended free sulphur particles of greater than colloidal size, comprising heating and mixing together until solution is effected an oil vehicle and a small amount of a suitable elastic-gel-forming substance substantially insoluble therein at normal temperatures, cooling said mixture without agitation until a gel is formed, and distributing powdered sulphur of greater than colloidal size throughout the gel by mixing together, said mixing rendering the gel freely flowing and said gel-forming substance being in sufficient amount to cause said sulphur to be stably suspended.

13. A cutting lubricant gel freely flowing at ordinary temperatures comprising an oil vehicle gelled with a small amount of soap and containing powdered sulphur of greater than colloidal size distributed therethrough in amount to function as a lubricating ingredient and be stably suspended therein.

14. A cutting lubricant gel freely flowing at ordinary temperatures comprising an oil vehicle gelled with a small amount of an alkali-soap and having powdered sulphur of greater than colloidal size distributed therethrough in amount to function as a lubricating ingredient and be stably suspended therein.

15. A cutting lubricant gel freely flowing at ordinary temperatures comprising an oil vehicle and sodium oleate soap and having powdered sulphur of greater than colloidal size distributed therethrough in sufficient amount to function as a lubricating ingredient, said soap being in sufficient amount to cause said sulphur to be stably suspended but not to prevent free flow of said lubricant under normal working conditions.

16. A cutting lubricant gel freely flowing at ordinary temperatures comprising an oil vehicle and heavy metallic soap and having powdered sulphur of greater than colloidal size distributed therethrough in sufficient amount to function as a lubricating ingredient, and stably suspended therein, said soap being in sufficient amount to cause said sulphur to be stably suspended but not to prevent free flow of said lubricant under normal working conditions.

17. A cutting lubricant gel freely flowing at ordinary temperatures comprising an oil vehicle and a lime rosin oil soap and having powdered sulphur of greater than colloidal size distributed therethrough in sufficient amount to function as a lubricating ingredient, said soap being in sufficient amount to cause said sulphur to be stably suspended but not to prevent free flow of said lubricant under normal working conditions.

18. A cutting lubricant gel freely flowing at ordinary temperatures comprising a mineral oil vehicle gelled with about 1% of sodium oleate soap and having about 5% of

powdered sulphur of greater than colloidal size distributed therethrough and stably suspended therein.

19. A cutting lubricant freely flowing at ordinary temperatures consisting of an oil vehicle and an oil and soap gel distributed therethrough and carrying in stable suspension dispersed free sulphur particles of greater than colloidal size in sufficient amount to function as the lubricating ingredient thereby permitting exceptionally high speed cutting, and said soap serving to minimize the corrosive action of the sulphur when the latter is not actually being employed to produce lubrication of the cutting tool where it engages the work.

20. The method of preparing a freely flowing cutting lubricant gel containing powdered sulphur of greater than colloidal size stably suspended in an oil vehicle, comprising mixing and heating together until solution is effected an oil vehicle and a small amount of soap, cooling said mixture and allowing a gel to form, and distributing powdered sulphur of greater than colloidal size throughout the gel by mixing therewith, said mixing rendering the gel freely flowing and said soap being in sufficient amount to cause said sulphur to be stably suspended.

21. The method of preparing a freely flowing cutting lubricant gel containing powdered sulphur of greater than colloidal size stably suspended in an oil vehicle, comprising mixing and heating together until solution is effected an oil vehicle and a small amount of alkali-soap, cooling said mixture and allowing a gel to form, and distributing powdered sulphur of greater than colloidal size throughout the gel by mixing therewith, said mixing rendering the gel freely flowing and said soap being in sufficient amount to cause said sulphur to be stably suspended.

22. The method of preparing a freely flowing cutting lubricant gel containing powdered sulphur of greater than colloidal size stably suspended in an oil vehicle, comprising mixing and heating together until solution is effected an oil vehicle and a small amount of heavy metallic soap, cooling said mixture and allowing a gel to form, and distributing powdered sulphur of greater than colloidal size throughout the gel by mixing therewith, said mixing rendering the gel freely flowing and said soap being in sufficient amount to cause said sulphur to be stably suspended.

23. The method of preparing a freely flowing cutting lubricant gel containing powdered sulphur of greater than colloidal size stably suspended in an oil vehicle, comprising mixing and heating together until solution is effected an oil vehicle and a small amount of lime rosin oil soap, cooling said mixture and allowing a gel to form, and distributing powdered sulphur of greater than

colloidal size throughout the gel by mixing therewith, said mixing rendering the gel freely flowing and said soap being in sufficient amount to cause said sulphur to be stably suspended.

24. The method of preparing a freely flowing cutting lubricant gel containing powdered sulphur of greater than colloidal size stably suspended in an oil vehicle, comprising mixing and heating together until solution is effected an oil vehicle and a small amount of sodium oleate soap, cooling said mixture and allowing a gel to form, and distributing powdered sulphur of greater than colloidal size throughout the gel by mixing therewith, said mixing rendering the gel freely flowing and said soap being in sufficient amount to cause said sulphur to be stably suspended.

25. The method of preparing a freely flowing cutting lubricant gel containing powdered sulphur of greater than colloidal size stably suspended in an oil vehicle, comprising mixing together a mineral oil and about 1% of sodium oleate soap, agitating at 300°-350° F. until solution is effected, cooling and allowing a gel to form, and distributing about 5% of powdered sulphur of greater than colloidal size throughout the gel by mixing therewith.

In testimony whereof, I have signed my name to this specification.

VICTOR R. ABRAMS.

100

105

115

120

125

130